

# UNITED STATES PATENT OFFICE.

GUSTAV SPITZ, OF BRÜNN, AUSTRIA-HUNGARY, ASSIGNOR TO GOLDSCHMIDT DETINING COMPANY, OF NEW YORK, N. Y., A CORPORATION OF NEW JERSEY.

## PROCESS OF MAKING PURE OXID OF TIN.

1,119,547.

Specification of Letters Patent.

Patented Dec. 1, 1914.

No Drawing.

Application filed November 6, 1909. Serial No. 526,805.

*To all whom it may concern:*

Be it known that I, GUSTAV SPITZ, subject of the Emperor of Austria-Hungary, and resident of Brünn, in the Empire of Austria-Hungary, have invented a new and useful Process of Making Pure Oxid of Tin, of which the following is an exact specification.

The present invention relates to a process of making pure oxid of tin from tin containing or holding materials of any kind, as for instance tin-plate waste, alloys of tin and the like.

Hitherto oxid of tin has generally been produced by burning metallic tin, but this method caused great losses in the furnace, both by volatilization and by the formation of slag. A somewhat pure oxid of tin has been obtained by treating tin with nitric acid, but the color of this oxid was yellow and not white, so that it could not be used, for instance, for enamels.

According to the present invention it is possible to obtain a pure oxid of tin, with the losses reduced to a minimum and practically negligible.

The process consists in placing the tin-containing or retaining materials, for instance, tin-plate waste of any kind, in a closed vessel and heating them with alkaline solutions, for instance of caustic soda, under high pressure and with the addition of an oxydizing material, whereby all the tin dissolves as stannate of sodium, the zinc as zincate and the lead as plumbate of sodium, while the impurities remain undissolved and sink to the bottom. From the solution of stannate of sodium thus obtained, the insoluble parts are removed and the lead is precipitated by chemical methods, for instance by tin, and the zinc by sulfid of sodium for instance. The solution of stannate of sodium, from which the settled foreign metals have been separated, is further treated with carbonic acid, boric acid or other acids or acid salts. Thus an oxid of tin is obtained which shows a clear white color but which still contains a small amount (from two to three per cent.) of alkali. These last traces of alkali cannot be removed by washing with water, they adhere to the product and thus render it useless for many technical purposes, as, for instance, for the manufacture of enamel. By numerous experiments I have found that the alkali is entirely removed by calcining the oxid

of tin after it has been subjected to a washing process, then grinding it if necessary, then washing it with a dilute acid or with a solution of a salt of ammonium, and finally drying it. When using nitric acid, the last traces of salts of lead and zinc, and even of salt of copper, may be removed by washing. To remove the last traces of alkali it is necessary to calcine the oxid of tin previously. Grinding is only necessary when the oxid of tin has become hard by the calcining, which will be the case, if alkali is still present.

In order to properly calcine the oxid of tin, it is necessary that it be heated to a high temperature, a red-white heat. It will not be sufficient to slightly heat the product for the mere purpose of drying, but it must be heated up to a degree of temperature, as stated, corresponding to red-white heat.

Oxid of tin which is to be employed in the manufacture of enamels must have the following qualities: It must be in a very finely divided state, amorphous, free from alkali and water and of a pure white color. In order to obtain such a product, it is necessary to add to the solution of stannate of sodium the precipitating medium in such a manner that the oxid of tin has no time to become crystalline, that is to say, the precipitating medium must be added so quickly and in such a quantity that the oxid of tin does not separate gradually but all at once. For this purpose it is best not to introduce gaseous carbonic acid into the boiling solution, as is usually done, but preferably to introduce solid bicarbonate, and simultaneously to agitate the fluid. It is advantageous if there are present in the liquid the various organic substances comprised in the waste materials and especially organic substances contained in old cans or boxes, for if such substances are present the separation of the oxid of tin in a finely divided state is facilitated. It is only possible to use an aqueous solution of bicarbonate of soda as precipitating medium, if the solution is introduced under a certain pressure, as otherwise an aqueous solution of bicarbonate of soda will become decomposed before boiling. In this case the solution of stannate of sodium, from which the foreign metals, etc., have been removed, is heated in a closed vessel, connected with a second closed vessel, in which latter vessel a solution of bicarbonate of

60

65

75

80

85

90

95

100

105

110

soda has been prepared by introducing carbonic acid under pressure into a solution of carbonate of sodium of say 40 degrees centigrade, while agitating the fluid. The solution of bicarbonate of soda thus prepared is under a pressure of say about 4 atmospheres while the stannate solution is under a pressure of say about 2 atmospheres. The stannate solution, under the pressure of 2 atmospheres, is heated up to 125 degrees centigrade, after which the solution of bicarbonate of soda is admitted, being under a pressure of 4 atmospheres and the temperature having been raised to say from 50 to 60 degrees centigrade by the absorption of carbonic acid. Oxid of tin is immediately precipitated in a finely divided amorphous state which renders it useful for enameling purposes. Naturally it is possible to similarly obtain oxid of tin from any stannate solution, as, for instance, from those solutions which are obtained in the electrolytic process of treating tin plate scraps in an alkaline bath.

According to the present process a perfectly white, finely divided powder of oxid of tin (99.5 to 99.9 per cent.  $\text{SnO}_2$ ) may be obtained. In order to remove traces of silica which may have entered the oxid of tin from the material treated, it may be advantageous to wash with hydrofluoric acid or solutions of fluorid of ammonium. As an example, oxid of tin is taken which, after having been dried and calcined still contains about 35 per cent. of  $\text{Na}_2\text{O}$  in form of basic salts. For neutralizing this small percentage of  $\text{Na}_2\text{O}$ , about 12 per cent. of marketable nitric acid would be required, but as other deleterious bodies may be present in the oxid of tin, as, for instance, oxid of zinc and oxid of lead, which also are soluble in nitric acid, it is necessary to have an excess of nitric acid in proportion to the amount of these bodies, that is to say, for instance, 20 kilograms or more of nitric acid may be employed with 100 kilograms of the above  $\text{SnO}_2$ . The solution is boiled with fresh steam, and the precipitate is filtered off, washed in the manner described and dried.

In my U. S. applications Ser. Nos. 526,603, and 526,604, I have described and claimed matters similar to those set forth in this application, and do not wish to be understood as here claiming the subject matters of said Serial Nos.

What I claim is:

1. The process of producing pure tin oxid in the most amorphous condition possible, from stannate solutions, which consists in precipitating the tin oxid and calcining it unmixed with acid.
2. The process of producing pure tin oxid in the most amorphous condition possible, from stannate solutions, which consists in precipitating the tin oxid, washing the pre-

cipitate with water and calcining it unmixed with acid.

3. The process of producing pure tin oxid in the most amorphous condition possible, from stannate solutions, which consists in precipitating the tin oxid, washing the precipitate with water, calcining it unmixed with acid, and then washing said calcined precipitate.

4. The process of producing pure tin oxid in the most amorphous condition possible, from stannate solutions, which consists in removing from these solutions other metals which contaminate them, precipitating the tin oxid, washing the precipitate with water and calcining it unmixed with acid.

5. The process of producing pure tin oxid in the most amorphous condition possible, from stannate solutions, which consists in removing from the solutions other metals which contaminate them, precipitating the tin oxid, washing the precipitate with water, calcining it unmixed with acid, and then washing said calcined precipitate.

6. The step in the process of producing pure tin oxid in the most amorphous condition possible from a stannate solution, which consists in treating said solution with a solution of alkali bicarbonate under pressure.

7. The step in the process of producing pure tin oxid in the most amorphous condition possible from a stannate solution, which consists in treating said solution with a solution of alkali bicarbonate under pressure while agitating the solution.

8. In the process of producing pure tin oxid in the most amorphous condition possible from a stannate solution, treating said solution under pressure with a solution of alkali bicarbonate under a higher pressure while agitating the solution.

9. The process of producing pure tin oxid in the most amorphous condition possible from a stannate solution, which consists in precipitating the tin oxid by means of a solution of alkali bicarbonate under pressure, and then calcining the precipitate.

10. The process of producing pure tin oxid in the most amorphous condition possible from a stannate solution, which consists in precipitating the tin oxid by means of a solution of alkali bicarbonate under pressure while agitating the solution, and then calcining the precipitate.

11. The process of producing pure tin oxid in the most amorphous condition possible from a stannate solution, which consists in precipitating the tin oxid by means of a solution of alkali bicarbonate under pressure while agitating the solution, then washing the precipitate with water, and calcining it unmixed with acid.

12. The process of producing pure tin oxid in the most amorphous condition possible, from stannate solutions, which consists in precipitating the tin oxid by

means of a solution of alkaline bicarbonate which has been separately prepared by introducing carbonic acid into a solution of carbonate of alkali under pressure, 5 while agitating the fluid, then washing the precipitate with water and calcining it.

13. The process of producing pure tin oxide in the most amorphous condition possible, from stannate solutions, which consists in precipitating the tin oxide by means of a solution of alkali bicarbonate under pressure, while agitating the fluid, then washing the precipitate with water, calcining it unmixed with acid, and then washing 5 said calcined precipitate.

14. The process of producing pure tin oxide in the most amorphous condition possible from stannate solutions, which consists in precipitating the tin oxide, washing the precipitate with water, calcining it at a red white heat unmixed with acid, and then washing said calcined precipitate.

15. The process of producing pure tin oxide in the most amorphous condition possible, from stannate solutions, which consists in precipitating the tin oxide by means of a solution of alkali bicarbonate under pressure, while agitating the fluid, then washing the precipitate with water, calcining 0 it at a red-white temperature unmixed with acid, and then washing the calcined precipitate.

16. The process of producing pure and clear white amorphous tin oxide from a stannate solution, which consists in precipitating tin oxide, and converting the impurities in said precipitate into readily removable form.

17. The process of producing pure and clear white amorphous tin oxide from an impure stannate solution, which consists in removing other metals that contaminate it, then precipitating the tin oxide, and then separating the remaining impurities from said precipitate.

18. The process of producing pure and clear white amorphous tin oxide from a solution of an alkaline stannate, which consists in treating said solution to precipitate the tin oxide, and then separating the alkali from said precipitate.

19. The process of producing pure and clear white amorphous tin oxide from a solution of an alkaline stannate, which consists in treating said solution to precipitate the tin oxide, washing said precipitate to remove the major portion of the alkali, and then subjecting said precipitate to treatment suitable for converting the residual alkali into 5 readily removable form.

20. The process of producing pure and clear white amorphous tin oxide from an impure solution of an alkaline stannate, which consists in removing from said solution other metals that contaminate it, then treating said

solution to precipitate the tin oxide, and then converting the alkali in said precipitate into readily removable form.

21. The process of producing pure and clear white amorphous tin oxide from a solution of an alkaline stannate containing metallic and organic impurities, which consists in removing from said solution other metals that contaminate it, then treating said solution to precipitate the tin oxide, and then separating the organic impurities and converting the alkali in said precipitate into 70 readily removable form.

22. The process of producing pure and clear white amorphous tin oxide from a solution of an alkaline stannate containing metallic and organic impurities, which consists in removing from said solution other metals that contaminate it, then treating said solution to precipitate the tin oxide, calcining 75 said precipitate, and then washing said calcined precipitate to remove the residual impurities.

23. The process of producing pure and clear white amorphous tin oxide from a solution of an alkaline stannate containing metallic and organic impurities, which consists in removing from said solution other metals that contaminate it, then treating said solution to precipitate the tin oxide, calcining 85 said precipitate, and washing said calcined precipitate with a solvent of silica.

24. The process of producing pure and clear white amorphous tin oxide from a solution of an alkaline stannate containing metallic and organic impurities, which consists in removing from said solution other metals that contaminate it, then treating said solution to precipitate the tin oxide, and then separating the organic impurities and converting the alkali in said precipitate into 90 readily removable form.

25. The process of producing pure and clear white amorphous tin oxide from an alkaline stannate solution, which consists in suddenly subjecting said solution to the action of a reagent suitable for precipitating the tin oxide in the most amorphous condition possible, and then converting the alkali in said precipitate into 105 readily removable form.

26. The process of producing pure and clear white amorphous tin oxide from a solution of an alkaline stannate containing metallic and organic impurities, which consists in removing from said solution other metals that contaminate it, then suddenly subjecting said solution to the action of a reagent suitable for precipitating the tin oxide in the most amorphous condition possible, and then separating the organic impurities and converting the alkali in said precipitate into 110 readily removable form.

27. The process of producing pure amorphous tin oxide from a stannate solution con- 120

taining organic impurities, which consists in precipitating the tin oxide substantially instantaneously from said solution, and calcining said precipitate unmixed with acid.

5 28. The process of producing pure amorphous tin oxide from tin-scrap containing organic impurities, which consists in subjecting said material to the action of a suitable detinning solution, removing from the resulting stannate solution other metals that contaminate it, precipitating the tin oxide from the resulting stannate solution containing organic impurities, and calcining said precipitate unmixed with acid.

10 29. The process of producing pure amorphous tin oxide from tin-scrap containing organic impurities, which consists in subjecting said material to the action of a suitable detinning solution, removing from the resulting stannate solution other metals that contaminate it, precipitating the tin oxide substantially instantaneously from the resulting stannate solution containing organic impurities, and calcining said precipitate unmixed with acid.

15 30. The process of producing pure amorphous tin oxide from a stannate solution containing metallic and organic impurities, which consists in removing from said solution other metals that contaminate it, precipitating tin oxide from said solution containing organic impurities, and calcining said precipitate unmixed with acid.

20 31. The process of producing pure amorphous tin oxide from a stannate solution containing metallic and organic impurities, which consists in removing from said solution other metals that contaminate it, precipitating tin oxide from said solution containing organic impurities, calcining said precipitate unmixed with acid, and washing said calcined precipitate with acid.

25 32. The process of producing pure and clear white amorphous tin oxide from an alkaline stannate solution containing organic impurities, which consists in precipitating the tin oxide from said solution, and then separating the organic impurities and alkali from said precipitate.

30 33. The process of producing pure and clear white amorphous tin oxide from a tin-containing material, which consists in subjecting said material to the action of an alkaline solution containing an oxidizing material, removing from the resulting stannate solution other metals that contaminate it, precipitating the tin oxide from said stannate solution, and converting the alkali in said precipitate into readily removable form.

35 34. The process of producing pure amorphous tin oxide from a tin-containing material, which consists in subjecting said material to the action of an alkaline solution containing an oxidizing material, remov-

70  
75  
80  
85  
90  
95  
100  
105  
110  
115  
120  
125  
130

ing from the resulting stannate solution other metals that contaminate it, precipitating the tin oxide from said stannate solution, and calcining said precipitate unmixed with acid.

35. The process of producing pure amorphous tin oxide from a tin-containing material, which consists in subjecting said material at high pressure to the action of an alkaline solution, removing from the resulting stannate solution other metals that contaminate it, precipitating the tin oxide from said stannate solution, and converting the alkali in said precipitate into readily removable form.

36. The process of producing pure amorphous tin oxide from a tin-containing material, which consists in subjecting said material at high pressure to the action of an alkaline solution, removing from the resulting stannate solution other metals that contaminate it, precipitating the tin oxide from said stannate solution, and calcining said precipitate unmixed with acid.

37. The process of producing pure amorphous tin oxide from a stannate solution, which consists in precipitating the tin oxide from said solution, calcining said precipitate unmixed with acid, grinding said calcined precipitate, and then washing said precipitate.

38. The process of producing pure amorphous tin oxide from a stannate solution containing substantially no metallic contaminations, which consists in precipitating the tin oxide substantially instantaneously from said solution, and calcining said precipitate unmixed with acid.

39. The process of producing pure amorphous tin oxide from a stannate solution, which consists in precipitating the tin oxide from said solution, calcining said precipitate unmixed with acid, and washing said precipitate with dilute acid.

40. The step in the process of obtaining pure and clear white amorphous tin oxide, which consists in separating the alkali from a precipitated amorphous oxid of tin-containing alkali.

41. The step in the process of producing pure and clear white amorphous tin oxide, which consists in converting into readily removable form the alkali in a precipitated oxid of tin containing alkali.

42. The step in the process of obtaining pure and clear white amorphous tin oxide, which consists in calcining unmixed with acid, a precipitated amorphous oxid of tin containing alkali.

43. In the process of producing pure and clear white tin oxide, washing a precipitated oxid of tin containing alkali, and then converting into readily removable form the alkali in said precipitate.

44. In the process of producing pure tin

- oxid, washing a precipitated oxid of tin containing alkali, calcining said precipitate unmixed with acid, and washing said calcined precipitate.
- 5 45. In the process of producing pure tin oxid, washing a precipitated oxid of tin containing alkali, calcining said precipitate unmixed with acid, and washing said calcined precipitate with acid.
- 10 46. In the process of producing pure and clear white tin oxid, separating the organic impurities from a precipitated oxid of tin containing alkali and organic and metallic impurities, and then separating residual alkali and metallic impurities from said 15 precipitate.
47. In the process of producing pure tin oxid, calcining, unmixed with acid, a precipitated oxid of tin containing alkali, and then washing the calcined precipitate. 20
- In testimony whereof I have hereunto set my hand in presence of two subscribing witnesses.

GUSTAV SPITZ.

Witnesses:

AUGUST FUGGER,  
ALEXANDER WEINGARTNER.

Copies of this patent may be obtained for five cents each, by addressing the "Commissioner of Patents, Washington, D. C."